

Aug. 31, 1937.

F. W. SULLIVAN, JR., ET AL

2,091,399

SYNTHETIC LUBRICATING OILS

Original Filed March 15, 1929

2 Sheets-Sheet 1



Aug. 31, 1937.

F. W. SULLIVAN, JR., ET AL

2,091,399

SYNTHETIC LUBRICATING OILS

Original Filed March 15, 1929

2 Sheets-Sheet 2



Fig. 2

Inventors:  
Frederick W. Sullivan, Jr.  
Vanderveer Voorhees  
BY

Burr K. Brown  
ATTORNEY

## UNITED STATES PATENT OFFICE

2,091,399

## SYNTHETIC LUBRICATING OILS

Frederick W. Sullivan, Jr., and Vanderveer Voorhees, Hammond, Ind., assignors to Standard Oil Company, Chicago, Ill., a corporation of Indiana

Original application March 15, 1929, Serial No. 347,446. Divided and this application November 1, 1932, Serial No. 640,634

5 Claims. (Cl. 196—151)

This invention relates to hydrocarbon lubricating oils, and particularly to synthetic lubricating oils comprised mainly of groups of straight chain hydrocarbons resulting from the action of aluminum chloride or other equivalent polymerizing agent upon suitable straight chain hydrocarbon material, as hereinafter set forth. The invention is illustrated by the accompanying drawings, in which

10 Fig. 1 is a graph of the equation hereinafter set forth, defining the limiting relationship of cold test to viscosity of oils prepared in accordance with the present invention.

Fig. 2 shows by graphs the comparative viscosity-temperature curves of typical natural lubricant oils and oils prepared in accordance with the present invention.

In accordance with this invention, we employ as the source of hydrocarbon material what may be termed a high boiling product consisting largely or entirely of normal paraffin hydrocarbons. For example, we may use hydrocarbon waxes, which are now well understood to consist substantially of straight-chain paraffin hydrocarbons. This wax may suitably be paraffin wax which occurs in Pennsylvania and Mid-Continent crude petroleum or other waxy material, such as petrolatum, slop wax, ozokerite wax or other hydrocarbon waxes. It must be understood, however, that the term "straight-chain hydrocarbon material" is not limited to waxes, since it is obvious that in oils containing wax, there is undoubtedly present straight-chain material of similar character, but of smaller molecular weight so that they do not solidify as readily as the ordinary waxes.

Thus, it is well recognized that Pennsylvania oil, for example, gas oil, contains more normal paraffin hydrocarbon material than does a similar distillate derived from Mid-Continent crude petroleum, while the latter likewise contains more straight-chain material than do similar oils derived from Coastal crudes. We may define our high boiling normal paraffin hydrocarbon material as one containing a larger amount or percentage of normal paraffin hydrocarbons than does a similar representative Pennsylvania distillate oil, and containing substantial proportions of constituents having a boiling point under atmospheric pressure conditions exceeding 600° F. In order to convert this normal hydrocarbon material into lubricating oils, it is necessary to induce a combination of molecules or polymerization. Because of the well-known unreactive nature of the paraffin hydrocarbons it is first neces-

sary to convert these substances into a more active form. This may be done by subjecting the normal hydrocarbons to pyrolysis as will be hereinafter described.

In producing improved lubricating oils according to this invention, we first crack the high-boiling normal paraffin hydrocarbon material to produce a desired type of unsaturated hydrocarbons suitable for the desired reaction with aluminum chloride. The cracking operation is preferably carried out under low pressure, substantially vapor phase conditions, suitably at a temperature between 750 and 1100° F. and at pressures below 100 lbs. Higher pressures may be employed, however. In general, it is preferred to determine the optimum conditions for cracking to secure maximum yield of desired products from a given initial material; as variations of temperature and pressure may materially affect the ultimate yield.

The distillate from such a cracking process may be redistilled to give a fraction substantially free of waxy material. Thus, we find ordinarily that if the end-point of such fraction is carried much above 500° F. the lubricating oils produced therefrom have an undesirably high cold test. When a distillate of about 500° F. end-point is polymerized to a lubricating oil, this oil will contain no apparent wax. On reduction of the polymerized oil, both the light overhead and the high viscosity bottom will have a low cold test. If desired, the distillate from the cracking operation may be fractionated into several portions which may be separately polymerized to products containing higher proportions of lighter or heavier lubricant products according to the nature of the cracked fraction employed.

In polymerizing the cracked fraction we may suitably employ from 0.5 to 4% of anhydrous aluminum chloride, but excellent results may be secured with larger and occasionally with smaller proportions. We also prefer to conduct the polymerization at a temperature between 100° and 250° F. a longer period of time being required at lower temperatures and a higher yield of more viscous products being produced. During the polymerization the mixture is thoroughly agitated. Substantial yields are obtained in three or four hours at temperatures of 175° F. and higher, but it is preferred to prolong the time of reaction to 15 to 20 hours, and at lower temperatures to as long as 50 hours, in order to obtain the maximum yield of lubricating oil.

After polymerization, it is necessary to separate tar or aluminum chloride sludge from the

oil. Most of the tar settles on standing and can be drawn off, leaving a brown oil containing particles of suspended tar. In order to obtain oils of the best color and lowest Conradson carbon, it is desirable to remove the remaining suspended tar. This may suitably be done by filtering with a small quantity of adsorbent earth, such as clay fines, or by prolonged settling, for example, 48 hours at 100-150° F. The oil may then be washed with an alkaline solution, as a 5 to 10% solution of caustic soda, if neutralization is required. The oil is then reduced by steam and fire or vacuum distillation to remove light oils and naphtha leaving a lubricating residue which may be separated by distillation to yield lubricating oils of desired viscosity.

The invention will more readily be understood from the following detailed description of a specific example:

20 A wax product derived, such as slack wax or a sweat oil (for example 110-120 melt) from Mid-Continent oil, containing 85% of mineral wax, the remainder being oil, is vaporized and the vapors heated at atmospheric pressure to a temperature between 900 and 980° F. to bring about cracking. After cracking, the vapors are separated from tar and are fractionated and condensed to yield a distillate having an end-point of about 500° F. The tar is eliminated and the 25 intermediate condensate is recycled and cracked with the feed. It is preferred to operate to produce between 10 and 25% of distillate per pass. During this cracking operation, 28% of gas, 5% of tar and 67% of distillate by weight are produced.

To such distillate about 1 to 3% of anhydrous aluminum chloride is added and the charge is maintained at about 210° F. for about 18 hours with thorough stirring. At the end of this period, the stirring is stopped and the tar, which amounts to about 7 to 10% of the initial charging stock is allowed to settle and is removed.

The remaining oil is reduced with steam; about 10% of light distillate, 80% of oil of 90 viscosity (210° F.), and about 10% of tar are produced. The heavy oil has the following inspection, after filtering through a small quantity of clay to secure the desired color:

Gravity, 32.5° A. P. I.; flash, 500° F.; pour, 50 -25° F.; viscosity at 210° F., 90 sec. Saybolt; viscosity at 100° F. 850 to 900 sec. Saybolt; viscosity index 107-112; Conradson carbon 0.13%; color 2 N. P. A.

Of course, it must be understood that other lubricating oils may be produced by a suitable control of the distillation. Thus, we may take off 10% of light distillate; 27.6% of oil of viscosity between 85 and 105 sec. Saybolt at 100° F.; 3.3% of oil of viscosity between 250 and 275 sec. 60 Saybolt, at 100° F.; and leave a bottom consisting of 49% of oil of viscosity of 190 sec. Saybolt at 210° F. The inspection of this bottom after claying is as follows:

Gravity, 31° A. P. I.; flash, 620° F.; pour -5° F.; viscosity at 210° F. 190 sec. Saybolt; viscosity at 100° F., 3000 sec. Salbolt; Conradson carbon 0.33%; color, 4 N. P. A. The yields of the lubricating oils thus obtained, based on the wax charging stock, are 48.6% of 90 viscosity oil and 70 28% of 190 viscosity oil (viscosities at 210° F.).

The aluminum chloride sludge may be reused on fresh oil to be polymerized to effect the desired change in whole or in part. Thus the 75 cracked distillate treated may first be subjected

to the action of sludge from previous treatment, and subsequently, to the action of fresh anhydrous aluminum chloride. The sludge resulting from the latter step may then be used in treating fresh distillate.

The oils produced according to the present invention possess remarkable properties which distinguish them from all lubricating oils known to applicants. Thus, we can produce oils which have a substantially better viscosity-temperature gradient than Pennsylvania lubricating oils, which possess very remarkable cold test properties and show a low Conradson carbon test. The viscosity temperature gradient is indicated by the viscosity index calculated by the method of 15 Dean & Davis described in Chemical and Metallurgical Engineering, 1929, vol. 36, pg. 618.

As indicated above many of the new oils produced according to our invention possess a lower temperature co-efficient of viscosity and a higher viscosity index than Pennsylvania lubricating oils. It will be understood that oils of various degrees of viscosity can be produced which will have a viscosity-temperature gradient less than that of a Pennsylvania oil of similar viscosity. For convenience, we will give the Saybolt viscosity of various oils at two arbitrary temperatures, viz. 100° F. and 210° F. and will compare the viscosity change with a standard Pennsylvania lubricating oil of the same viscosity at the 20 lower temperature. Thus, with wax derived from Mid-Continent crude petroleum containing about 15 or 25% of oil as starting material, the finished lubricating oil has a viscosity-temperature gradient substantially the same as that of Pennsylvania lubricating oil. With higher percentages of wax the lubricating oil has a lower temperature co-efficient of viscosity than Pennsylvania as indicated by the specific example given above, while an even better gradient is obtained with more purified wax. With a paraffin base oil which is richer in straight line hydrocarbon material than is Mid-Continent oil, the effect of oil content of the wax is not so marked.

It must be understood that our invention is not limited to oils having a viscosity-temperature gradient better than Pennsylvania oils, since it comprises many oils which have outstanding valuable properties, but which, nevertheless, may have a temperature co-efficient of viscosity equal to or not quite so good as Pennsylvania oil; an oil may be made having a lower temperature viscosity co-efficient than for example, a Mid-Continent lubricating oil and at the same time a cold test lower than a Coastal lubricating oil of the same viscosity at 100° F. with its normal wax content.

An important characteristic of our oils, both those superior to and somewhat inferior to Pennsylvania with respect to viscosity change with temperature is their low pour or solid points. This characteristic of our oils may suitably be expressed as follows:

$$S \leq 37.2 \log_{10} V_{100} - 134$$

Where S is the solid point in degrees Fahrenheit, and  $V_{100}$  is viscosity in seconds Saybolt at 100° F. The solid point, in the above formula, is 5° F. below the pour point, as determined by suitable methods. The logarithm in the equation is to the base 10. In Fig. 1 the equation  $S = 37.2 \log_{10} V_{100} - 134$  is plotted on semi-log coordinates, the abscissae representing the solid

point in degrees Fahrenheit and the ordinates the logarithms of the viscosity in seconds Saybolt at 100° F. The points S1, S2, S3 and S4 indicate the positions on the graph of the correspondingly designated oils of the present invention in the table hereinafter set forth.

In addition to these characteristics, our lubricating oils possess very low Conradson carbon tests, very good color and very high flash points. Thus, oils produced from material containing 85% wax and upward as starting material have substantially higher flash points than Pennsylvania lubricating oils of similar viscosity at a standard temperature.

In order to ascertain more definitely the nature of our products, we give the following examples of oils of the first class, that is lubricating oils produced by the present process having viscosity temperature gradients better than standard Pennsylvania or paraffin base lubricating oil of similar viscosity. These lubricating oils were produced substantially as described above, from the starting material indicated.

25

| 30 | Initial stock                | Lubricating oil of present invention |         |         |            |                  | Standard Pennsylvania lubricating oil |                           |            |       |
|----|------------------------------|--------------------------------------|---------|---------|------------|------------------|---------------------------------------|---------------------------|------------|-------|
|    |                              | Viscosity sec. Saybolt               |         |         | Cold test  | Gravity A. P. I. | Viscosity gravity constant            | Viscosity in sec. Saybolt |            |       |
|    |                              | V. I.                                | 210° F. | 100° F. |            |                  |                                       | At 210° F.                | At 100° F. | V. I. |
| 35 | S3 85% wax from M. C. crude. | 107.6-<br>112.1                      | 90      | 860-900 | °F.<br>-30 | 32.5             | 0.776                                 | 90                        | 950        | 103   |
|    | S4 85% wax from M. C. crude. | 190                                  | 2800    |         | -10        | 31               | 0.541                                 | P2 190                    | 3000       |       |
|    | S1 65% wax from M. C. crude. | 133                                  | 86      | 675     | -35        | 34               | 0.779                                 | P1 86                     | 860        | 104.8 |
|    | S2 Refined petrolatum wax    | 118.6                                | 87      | 735     | -36        | 34               | 0.760                                 | 87                        | 900        | 102.7 |

In Fig. 2 of the drawings, curves of the temperature-viscosity relationships of typical nature

properties within the aforesaid definitions, we give the following:

| 45 | Initial stock                                                                   | Lubricating oil of our process |         |         |            |                  | Standard Mid-Continent lubricating oil |                         |            |       |
|----|---------------------------------------------------------------------------------|--------------------------------|---------|---------|------------|------------------|----------------------------------------|-------------------------|------------|-------|
|    |                                                                                 | Viscosity sec. Saybolt         |         |         | Cold test  | Gravity A. P. I. | Viscosity gravity constant             | Viscosity, sec. Saybolt |            |       |
|    |                                                                                 | V. I.                          | 210° F. | 100° F. |            |                  |                                        | At 210° F.              | At 100° F. | V. I. |
| 50 |                                                                                 |                                |         |         |            |                  |                                        |                         |            |       |
| 55 | 65% wax from M. C. crude.....                                                   | 91.8                           | 77      | 804     | °F.<br>-20 | 29.4             | 0.800                                  | M1 77                   | 930        | 74.1  |
|    | 70% wax from M. C. crude.....                                                   | 103.4                          | 84      | 835     | -36        | 30.8             | 0.788                                  | M2 84                   | 1120       | 73.5  |
|    | 75% wax from M. C. crude.....                                                   | 101                            | 83      | 840     | -20        | 30.9             | 0.788                                  | 83                      | 1100       | 72.7  |
|    | Paraffin; (vapor phase cracked; distillate of 200° F. end-point).....           | 87.3                           | 88      | 1083    | -25        | 31.5             | 0.719                                  | 88                      | 1220       | 74.4  |
|    | Paraffin; (vapor phase cracked distillate boiling between 200 and 310° F.)..... | 96.2                           | 85      | 926     | -25        | 31.3             | .....                                  | 85                      | 1150       | 73.4  |

oils are shown, the abscissae representing viscosities in seconds Saybolt at 210° F. and the ordinates representing viscosities in seconds Saybolt at 100° F. on a logarithmic scale. The curve designated C is typical of Coastal oils; that designated MC, of Mid-Continent oils; that designated P of Pennsylvania oils, and that designated S of oils of the present invention. The points P1 and P2 designate the positions on the graph of the correspondingly marked Pennsylvania oils in the table above, and those marked S1, S2, and S4 of the correspondingly marked synthetic oils of the present invention in the table above.

These oils also have the specific gravity which characterize most of our oils.

In Fig. 2, the points M1 and M2 designate the positions on the graph of the Mid-Continent oils in the above table having the corresponding markings and the point M3 designates a typical Mid-Continent oil of a viscosity of 152 sec. Saybolt at 210° F. and 3200 sec. Saybolt at 100° F. described by Gruse, Petroleum and its Products, published 1928, on pg. 267.

Although the present invention has been described in connection with the details of specific examples thereof, it must be understood that such details are not intended to be limitative of the invention, except insofar as set forth in the

5

10

15

20

25

30

35

40

45

50

55

60

65

70

75

accompanying claims. For example, other means of activating normal paraffin hydrocarbons and wax may be employed besides cracking, and other methods of polymerizing these materials into lubricating oils are contemplated. We have discovered that these materials may be converted into lubricating oils with unprecedented properties, and we intend to include in the following claims, every product resulting from our discovery. This application is a division of our Patent No. 1,955,260.

We claim:

1. A synthetic hydrocarbon lubricating oil derived from straight chain hydrocarbon wax, 15 said synthetic oil being characterized by having its component molecules consisting predominately of groups of atoms which groups of atoms have substantially the same arrangement and weight as the polymerizable molecules in a fraction of cracked straight chain hydrocarbon wax, 20 which fraction has a boiling range lower than wax, said synthetic oil having a viscosity index between about 91.8 and about 133, a solid point between about -10° F. and about -36° F., and 25 an A. P. I. gravity between about 29.4 and about 34 degrees.

2. A synthetic hydrocarbon lubricating oil derived from straight chain hydrocarbon wax, 30 said synthetic oil being characterized by having its component molecules consisting predominately of groups of atoms which groups of atoms have substantially the same arrangement and weight as the polymerizable molecules in a fraction of cracked straight chain hydrocarbon wax, which 35 fraction has a boiling range lower than wax, said synthetic oil having a viscosity index between about 91.8 and about 133, a viscosity between about 95 and about 3,000 seconds Saybolt at 100° F. and an A. P. I. gravity between about 29.4 40 and about 34 degrees.

3. A wax-free synthetic hydrocarbon lubricating oil derived from straight chain hydrocarbon wax, 45 said synthetic oil being characterized by having its component molecules consisting predominately of groups of atoms which groups of atoms have substantially the same arrangement and weight as the polymerizable molecules in a fraction of cracked straight chain hydro-

carbon wax, which fraction has a boiling range lower than wax, said synthetic oil having a viscosity index between about 91.8 and about 133, an A. P. I. gravity between about 29.4 and about 34 degrees, a solid point between about -36° F. and the maximum value,

$$37.2 \log_{10} V_{100} - 134$$

where  $V_{100}$  is the viscosity in seconds Saybolt at 100° F. and the solid point is expressed in degrees Fahrenheit.

4. A substantially wax-free synthetic hydrocarbon lubricating oil derived from paraffin wax by converting the wax into normally liquid polymerizable compounds, of lower molecular weight than the wax and of the nature of straight chain fragments of the wax, and thereafter treating with a polymerizing catalyst, thereby producing hydrocarbons of higher molecular weight, said lubricating oil being essentially composed of molecules which are polymers of normally liquid compounds of the nature of straight chain fragments of the paraffin wax, said oil being characterized further by a viscosity at 210° F. between about 83 and about 190 Saybolt, a proportionately increasing viscosity at 100° F. of between about 840 and about 3,000 Saybolt and a solid point between about -36° F. and the maximum value indicated by the relation  $37.2 \log_{10} V_{100} - 134$  wherein  $V_{100}$  is the Saybolt viscosity at 100° F. and the solid point is expressed in degrees Fahrenheit.

5. A synthetic hydrocarbon lubricating oil derived from straight chain hydrocarbon wax, 35 said synthetic oil being characterized by having its component molecules consisting predominately of groups of atoms which groups of atoms have substantially the same arrangement and weight as the polymerizable molecules in a fraction of cracked straight chain hydrocarbon wax, 40 which fraction has a boiling range lower than wax, said synthetic oil having a viscosity between about 835 and about 3,000 Saybolt at 100° F., a viscosity index between about 101 and about 133 and a viscosity gravity constant between about 0.760 and about 0.541.

FREDERICK W. SULLIVAN, JR.  
VANDERVEER VOORHEES.